

Patented Oct. 16, 1928.

1,687,924

# UNITED STATES PATENT OFFICE.

CHRISTOPHER H. BIERBAUM, OF BUFFALO, NEW YORK, ASSIGNEE TO LUMEN BEARING COMPANY, OF BUFFALO, NEW YORK, A CORPORATION OF NEW YORK.

## BEARING ALLOY.

No Drawing.

Application filed June 4, 1926. Serial No. 113,829.

This invention relates more particularly to alloys used for bearings.

It is well known, and experience has amply proven, that a single homogeneous metal is not suited for bearing purposes, and that the first requirement for a bearing metal is that it be an alloy composed of at least two metals, or a metal and a metalloid, which shall have at least a limited degree of solubility while in the molten state; but that upon cooling it shall partially separate out into dissimilar crystals and thus form the requisite micro-structure, which is necessary in all bearing alloys. It is not only necessary that a bearing metal shall be composed of chemically dissimilar crystals, but it is all important that these crystals shall have a marked degree of difference in their physical hardness and wearing qualities.

It is essential that all bearing metals should be alloys having two or more phases: that is, that they consist of hard and relatively soft microscopical particles intimately mixed. The function of the hard particles or bearing crystals, is to support the load and resist the wear when actual metallic contact exists between the bearing surfaces. The functions of the softer particles are to allow the harder particles to adjust themselves to surface requirements of the journals and to wear down slightly below the surface of the harder, thereby forming slight depressions, on the apparently smooth wearing surface of the bearing, in which depressions minute quantities of the lubricant are held at such times when the bearing surfaces are brought into actual metallic contact with each other. It is this characteristic of certain alloys to form these slight depressions and thus provide the means for retaining a residual amount of the lubricant, that characterizes them as true bearing metals.

The wide range of hardness between the hardest crystal and the softest crystal in a bearing metal determines its value as such. However, the hardest crystal should at no time be hard enough so as to prove distinc-tively abrasive to the journal, nor should the softest crystal be soft enough to cause it to flow within the body of the metal when the same is in service.

An alloy which perhaps most characteristically represents a bearing metal is one composed of copper and tin, containing sufficient tin to produce the tin-copper eutectoid

or delta crystal. Now, it is a well known fact in metallurgy that this copper-tin alloy containing sufficient tin to produce the eutectoid under ordinary foundry conditions, that chilling or rapidly cooling of the same from the molten to the solid increases the physical strength of this alloy and that by such chilling, the amount of the eutectoid formed is decreased and also that if, under extreme conditions, this alloy is chilled sufficiently sudden no eutectoid is formed.

In the heated molten state the tin is evenly diffused in the copper. As cooling begins the tin tends to separate from the copper so that the first solidification in the copper is rich in alpha crystal. If cooling progresses slower, the tin has time to more completely separate from the copper, with the result that slower cooling produces a softer alpha and a larger amount of the delta crystal, thus effecting characteristics best suited for a bearing metal. On the other hand, chilling hardens the alpha crystal by retaining a larger amount of tin in solid solution within the same and, likewise, chilling decreases the aggregate amount of the brittle delta crystal; thus, for two reasons, chilling increases the strength and physical properties of this alloy but decreases its value as a bearing metal.

The standard alloy now commonly used in the worm wheels for automotive drives and for power reduction gears is composed of 89 percent copper and 11 percent tin, together with a small quantity of the deoxidizing agent, such as phosphorus, manganese or the like. This latter constituent is so small that it need not be given further consideration here.

In general service, in both the United States and Europe, these worm wheels are cast upon a chill around their periphery for the purpose of producing in that part of the casting a high tensile strength, since it is this periphery where the teeth are cut that engages with the driving worm.

I have discovered that with the addition of a percentage of nickel to this standard copper-tin alloy, when made in the usual way, that three distinct advantages obtain: an improvement in the strength and elastic limit of the alloy, a marked increase in the bearing value of the same and the production of an alloy admirably adapted for casting in a metal mold.

The advantage secured by the addition of

a relatively small percentage of nickel to this alloy is due to the high fusing point of the same and the fact that the atomic volume of nickel is so nearly equal to that of copper and the grouping of the nickel atoms corresponds to that of copper, both having the cubic face centered lattice structure; this together with the fact that the atomic volume of tin is more than double that of copper and that the natural grouping of the tin atoms differs from that of copper, it being the body centered tetragonal lattice structure. For these reasons, when the three metals are in a molten state, the atoms of the one having the highest fusing temperature tend to orient themselves first, thus causing the nickel to replace the tin and forming an alpha or first solidifying crystal, which contains a much lower percentage of tin than would exist without the nickel present, and for the reason that the atomic grouping of nickel and copper are so nearly identical, a small percentage of nickel in the copper has a less hardening effect upon the same than a corresponding amount of tin would have; therefore, a small percentage of nickel added to this copper-tin alloy results in the production of a softer alpha crystal and a larger aggregate amount of the hard delta crystal.

Nickel added to this alloy in varying amounts has a very distinct and pronounced effect on the formation of the delta crystal. In general, the presence of nickel causes an increase of the aggregate amount of the delta, it replacing the tin in the alpha crystal leaves a larger amount of the latter to enter the delta formation, at the same time causes it to form in a smaller or more finely subdivided state, a condition beneficial to a bearing metal. When making the alloy with  $\frac{1}{2}$  per cent of nickel a distinct effect is produced upon the eutectoid formation of the delta, and increasing from  $\frac{1}{2}$  to  $1\frac{1}{4}$  per cent the delta formation becomes more and more striated and lamellar, and at  $1\frac{1}{2}$  per cent the delta becomes solid or massive, assuming a complete noneutectoid form. This condition obtains for all percentages of nickel above  $1\frac{1}{2}$  per cent. The addition of nickel in all proportions thus produces an effect upon the delta crystal so as to increase its wear or abrasion resisting capacity.

This improved alloy has a very distinct advantage when used for castings made in metal or chill molds; in that it does not have the disadvantage or drawback which the standard alloy has. When pouring the standard alloy against a chill, the alpha crystal is hardened by the fact that a larger per cent of tin is held in solid solution in this crystal, and at the same time a much smaller amount of delta crystal is formed. The improved alloy does not possess these disadvantages for the reason that in the presence of the nickel the alpha crystal is not hardened by chilling,

and at the same time the delta crystal is not decreased in like amount, for which reasons the actual chilled surface of the improved alloy has a soft alpha crystal and a large amount of the delta formations upon the chilled surface. The improved alloy thus retains its full bearing value even though it is chilled, by retaining a wide range of hardness between the hardest and softest crystals.

It has been found in practice, that the minimum amount of nickel which can be used to advantage in this standard alloy is one-half of one percent, and that the largest amount of nickel that can be used to advantage is ten percent; when, however, such a large amount of nickel is used, it is permissible to cut down the percentage of tin to, say five percent, and still retain the beneficial effects upon the delta crystal, copper being the remaining constituent.

As the tin content of the alloy is varied, the percentage of nickel necessary to accomplish a certain transformation must be varied.

In practice varying amounts of lead are often added to the standard alloy, the lead having the effect of making the metal more plastic, a condition very desirable where conformability is necessary. The lead for all practical purposes is present in the form of a mechanical mixture and accordingly it may be added to this improved alloy in manner as heretofore with corresponding beneficial effects.

My invention is such that it can be readily practiced by any experienced foundryman versed in the art. The nickel is secured in the form of a copper-nickel alloy as commonly found on the market. The copper, together with the necessary percent of alloyed nickel is first melted, the deoxidized agent is then added, and finally the tin, after which lead may or may not be added as desired. My preferred composition is copper 84.5 percent, tin 10.5, nickel 5 percent.

It is to be understood that the word "bearing" as used in this application and in the appended claim is intended to include gear wheels, worm wheels and similar articles which require characteristics of hardness and wear resistance, as indicated hereinbefore.

I claim as my invention:

A bearing consisting of an alloy containing 84.5 percent copper, 10.5 percent of tin, and 5 percent of nickel; said alloy being cast in the absence of zinc against a chill so that the alpha crystal is not hardened but left soft and a large amount of hard delta crystal is formed upon the chilled surfaces, and a wide range of hardness being present between the hardest delta crystal and the softest alpha crystal.

In testimony whereof I hereby affix my signature.

CHRISTOPHER H. BIERBAUM.